

## 1

3,007,911

METHOD OF SULFOCHLORINATING  
HYDROCARBONS

Helen Sellei Beretvas, Chicago, and Robert S. Barnes, Jr., Olympia Fields, Ill., assignors to Standard Oil Company, Chicago, Ill., a corporation of Indiana  
No Drawing. Filed Dec. 2, 1958, Ser. No. 777,605  
21 Claims. (Cl. 260—139)

This invention relates to improvements in the sulfochlorination of unsaturated hydrocarbons. In particular, it relates to the treatment of unsaturated hydrocarbons with sulfur chloride to produce compositions having high sulfur content, high chlorine content, unusually light color, and high temperature color stability.

Sulfurization of unsaturated hydrocarbons has been effected in the past by processes which generally comprise the steps of sulfurization by reacting unsaturated hydrocarbons with sulfur chloride in the presence of added water at a temperature from about 80° F. to about 150° F., neutralization of the resulting product with an alkaline reagent such as an alkali metal or alkaline earth oxide, hydroxide or carbonate, and separation of the neutralization product from the hydrocarbon insoluble products by filtration. The products for such a process usually have a high sulfur content and a high chlorine content. It has now been found that high sulfur-high chlorine-containing hydrocarbon compositions can be obtained in a process which eliminates the time consuming neutralization step and allows completion of the process reactions within a minimum amount of time and without necessitating the handling of strong alkali materials. Furthermore, it has been found that by our present process hydrocarbons of unusually high sulfur content, light color and having excellent high temperature color stability, may be produced.

Therefore, an object of the present invention is to produce sulfochlorinated hydrocarbons having light color and excellent color stability at relatively high temperatures.

Another object of the present invention is to provide a process for sulfochlorinating unsaturated hydrocarbons which permits the elimination of time consuming neutralization steps.

A further object is to produce improved materials which may be employed as additives to cutting oils and gear oils and as intermediates for the preparation of additives for use in internal combustion motor oils, diesel oils, etc., and which impart extreme pressure characteristics to the oils in which they are used. Other objects and advantages will be apparent from the following.

Broadly stated, the present invention comprises the steps of sulfochlorinating a linearly unsaturated hydrocarbon by treatment with sulfur chloride, refluxing the sulfochlorinated hydrocarbon in the presence of a solvent and water mixture, and finishing the resulting refluxed material by removing undesirable and occluded matter. The linearly unsaturated hydrocarbons which may be sulfochlorinated in accordance with this invention are those unsaturated hydrocarbons having at least one double bond in a linear chain and are intended to include olefins, aromatics having unsaturated alkyl groups, cycloparaffins having unsaturated alkyl groups, partially unsaturated polymers, unsaturated acids, alcohols and esters,

## 2

etc. The olefins used in the present invention are those having from 6 to 18 carbon atoms and preferably from 7 to 12 carbon atoms. Synthol olefins prepared by Fischer Tropsch synthesis of carbon monoxide and hydrogen may also be used but it is advantageous to purify the raw synthol olefins by fractional percolation through Attapulgus clay, silica, alumina, etc., before sulfochlorination to get a product having less objectionable odor. The partially unsaturated polymers are those having linear unsaturation, such as partially unsaturated polymers prepared from acyclic olefins, monoolefins, aromatics having unsaturated alkyl groups and the like.

In carrying out the sulfochlorination in accordance with the present invention, an unsaturated hydrocarbon or a mixture of unsaturated hydrocarbons is treated with sulfur chloride. It has been found advantageous to carry the sulfur chloride treatment out in the presence of water to obtain a lighter colored product although water is not necessary to the sulfochlorination reaction. The sulfur chloride used may be any of the usual sulfur chlorides, such as sulfur monochloride, sulfur dichloride, or mixtures thereof. Because of its higher sulfur content, sulfur monochloride is preferred. In sulfochlorinating the unsaturated hydrocarbon in the presence of water we prefer to incrementally add the sulfur chloride and water simultaneously but separately to the unsaturated hydrocarbon. However, we have found that there are other acceptable procedures in conducting the reaction. The sulfochlorination may be carried out by incrementally adding the sulfur chloride to a mixture of the unsaturated hydrocarbon and water. In this case the sulfur chloride should be added slowly to keep the reaction from becoming too vigorous and so as not to exceed the boiling point of the mixture. Another method of sulfochlorination within the scope of the present invention is by adding the unsaturated hydrocarbons to a mixture of sulfur chloride and water. In this case special precaution must be taken to provide adequate cooling because the reaction is particularly vigorous. Following still another procedure, the water may be added to a mixture of sulfur chloride and unsaturated hydrocarbon, however, this procedure produces a product of darker color than that obtained by the other above mentioned technique and is therefore the least preferred procedure. If water is omitted, the sulfur chloride should be added slowly to the hydrocarbon. In any of the above procedures, agitating or mixing is advantageous to minimize localized vigorous reactions.

In accordance with the preferred sulfochlorination procedure, sulfur chloride and water are added simultaneously but separately to the unsaturated hydrocarbon, the sulfur chloride being added in molar amounts. In the present invention we use from about 0.3 to about 2.0 moles of sulfur chloride and if the unsaturated hydrocarbons are olefins preferably from about 0.4 to 0.8 mole of sulfur chloride per mole of unsaturated hydrocarbon. In the sulfochlorination reaction sufficient sulfur chloride is used to provide approximately 0.4 to 3.0 atoms of sulfur per unsaturated olefinic bond in the reacting hydrocarbon. When polymers are reacted generally more than 60% of the unsaturated polymer will react. Greater molar amounts of sulfur chloride per mole of hydrocarbon should be used with polymers having a large number of unsaturated bonds and where more highly unsaturated

olefins, such as diolefins, are used. Because the reaction is vigorous if allowed to proceed uninhibited from a total mixture of all reactants used, the sulfur chloride is added at a rate slow enough to maintain the exothermic reaction within a temperature range of about 0° C. to about 90° C. and preferably not exceeding 55° C. It is also advantageous to cool the separate reactants before combining them or to cool the reaction itself in order to maintain the reaction within the above temperature range. Allowing the temperature to exceed 90° C. will cause discoloration of the product and will also cause the reactants to flow from the top of the reactor where an open reactor is used. Even temperatures in excess of 55° C. may cause discoloration. The water is added separately during the sulfochlorination over a period of from about 10 to 45 minutes. We use from 1 to about 50 volume percent, preferably from about 5 to about 26 volume percent, of added water based on the unsaturated hydrocarbon. The addition of water is advantageous in that it improves the color stability of the sulfochlorinated product. The water also helps attain a more complete reaction. The sulfochlorination reaction is allowed to continue until complete, and the refluxing step is started immediately after the reaction is complete, i.e., immediately after the completion of reactant addition. Because the reaction is exothermic in nature, it is preferred to apply external cooling to the reaction mixture while the reaction proceeds. By applying external cooling, the period of time required for the reaction may be greatly decreased because removal of exothermic heat will allow faster addition of the reactants to the unsaturated hydrocarbon without producing problems of product discoloration. Following the preferred procedure as outlined above the sulfur chloride treatment may be completed within about one hour and should not take longer than about five or six hours.

During sulfochlorination it may become desirable to add an antifoam agent such as a silicone polymer or other suitable material to inhibit excessive turbulence and foaming of the reaction mixture.

Phosphorus sulfide such as  $P_2S_5$ ,  $P_4S_3$ ,  $P_4S_{10}$ , etc. may be advantageously incorporated in small amounts into the reactants of the present invention to further increase the color stability of the reaction products. The phosphorus sulfide apparently reacts with the unsaturated hydrocarbon during sulfochlorination and during the later reflux steps. We prefer to add the phosphorus sulfide during the sulfochlorination step before the addition of sulfur chloride because we have found that addition at this time produces a sulfochlorinated hydrocarbon of greater color stability. When phosphorus sulfide is added to the reactants, water may also be added to aid the reaction and further increase color stability. In carrying out the preferred procedure, we mix phosphorus sulfide with the unsaturated hydrocarbon prior to the addition of sulfur chloride. The amount of phosphorus sulfide added is in the range of from about .0025 mole to about 0.2 mole and preferably from about .005 to about .05 mole per mole of unsaturated hydrocarbon. Thus, the amount by weight of phosphorus sulfide used is dependent upon the molecular weight of the hydrocarbon. Accordingly, for example, we have found that sufficient phosphorus sulfide to give a product having 0.1 to 2.5 weight percent phosphorus based upon the weight of an unsaturated hydrocarbon having seven carbon atoms is used during sulfochlorination. When the phosphorus sulfide is added to the sulfochlorination reaction, it is advantageous to carry the reaction out in the presence of a nitrogen atmosphere to prevent flashes which may normally be caused by the phosphorus compound in the presence of air. It has been found that when phosphorus sulfide is added during the sulfochlorination step the reactants are more stable at higher temperatures and discoloration problems arising from uncontrolled temperatures in the reaction are substantially minimized.

Upon completion of the sulfochlorination of the olefin as set out above, the reaction product is refluxed, preferably immediately after sulfochlorination, at least once in the presence of a solvent and water mixture. Although the reaction product may be first removed from the unreacted components and impurities as by filtration or other known separating methods, we prefer to add the solvent and water mixture directly to the reaction mixture at the completion of sulfochlorination.

In the reflux step, total reflux of the mixture of reactants is effected so that all of the reactants as well as substantially all of the solvent and water are retained in the mixture with no appreciable amount of the reaction mixture being driven off with the exception of HCl. We use a water cooled refluxing condenser in the reflux step. The reflux is carried out at the total reflux temperature of the reaction mixture, which temperature normally will not exceed about 100° C. under atmospheric conditions, because of the presence of the water. The solvents which are useable in the solvent and water mixture are the oxygen-containing essentially non-reacting water-miscible organic compounds boiling below 100° C. and preferably above 50° C. The solvent may advantageously be a water-miscible ketone or alcohol. The water-miscible alcohols are preferred as solvents and of particular preference is isopropanol. Lower temperatures may be advantageously used down to about 65° C., at atmospheric pressure, such as when methanol is used as the solvent or even to about 55-60° C. as when acetone is used as the solvent. We prefer to reflux the reactants in the range of from about 75° C. to about 95° C. in the presence of a mixture of water and isopropanol, the solvent of particular preference. Of course, the above recited temperatures correspond to refluxing at substantially atmospheric pressure; changes in pressure may require changes in the temperature range and such changes are to be considered within the scope of the present invention. The reflux is continued for a sufficient period of time to eliminate labile chlorine as HCl. The period of time for refluxing is in the range of from about 10 minutes to about ten hours and preferably from about one-half hour to about four hours. During reflux, the loose chlorine from sulfochlorination is eliminated as HCl substantially dissolved in the water layer removed after refluxing. Reflux may be repeated one or more times and we have found that two refluxes of about one hour each are sufficient. When reflux is repeated, the water layer is separated from the reactants after reflux and a second reflux mixture of solvent and water is added to the reactants, preferably immediately. The total time of reflux when more than one reflux is used should fall within the above limits.

In the first refluxing, we prefer to use a mixture of about 50% solvent and about 50% water by volume and if a second or subsequent refluxing is used, we prefer to use a mixture of about 80% water and about 20% solvent by volume; however, any solvent and water mixture is suitable. The amounts of the mixture used may vary with the hydrocarbon starting material as well as the number of refluxes. For example, it has been found that 500 cc. of isopropanol and water mixture per 1000 grams of an olefin starting material is sufficient for the first refluxing and 250 cc. per 1000 grams is sufficient if subsequent refluxing is desired.

Refluxing with solvent and water eliminates the labile chlorine and other unreacted inorganic impurities left in the product from the sulfur chloride treatment step. The labile chlorine is eliminated in the form of hydrogen chloride and the severity, length and number of refluxes is partially determined by the amount of chlorine which needs to be eliminated from the product. The reflux also serves to increase the sulfur content of the product. If phosphorus sulfide is used during sulfochlorination, the phosphorus content of the product is also increased in comparison with a sodium hydroxide neutralized product,

supra. The increase of phosphorus and sulfur content can be readily understood by reference to the following comparison of analyses of products prepared in accordance with the present invention with those prepared by a process using neutralization of a sulfur chloride treated product with sodium hydroxide after eliminating unreacted olefins by blowing with nitrogen.

TABLE I

|                                     | Product Analysis |            |           | Phosphorus Compound Used During Sulfur Chloride Test |
|-------------------------------------|------------------|------------|-----------|------------------------------------------------------|
|                                     | Percent S        | Percent Cl | Percent P |                                                      |
| (1)                                 |                  |            |           |                                                      |
| Refluxed Product <sup>2</sup> ..... | 29.4             | 9.34       | 0.80      | 5% P <sub>4</sub> S <sub>3</sub> . <sup>3</sup>      |
| Do. <sup>2</sup> .....              | 30.6             | 8.8        | 0.69      | 5% P <sub>4</sub> S <sub>3</sub> .                   |
| NaOH Treated Product.....           | 25.8             | 14.1       | 0.33      | 5% P <sub>4</sub> S <sub>3</sub> .                   |
| Do.....                             | 25.8             | 10.7       | 0.20      | 5% P <sub>4</sub> S <sub>3</sub> .                   |
| Do.....                             | 23.2             | 15.8       | -----     | None.                                                |

<sup>1</sup> All products above before reflux or NaOH neutralization as indicated were prepared by sulfochlorinating a C<sub>7</sub> olefin with 70 gm. S<sub>2</sub>Cl<sub>2</sub> per 100 gm. C<sub>7</sub> olefin in the presence of H<sub>2</sub>O.

<sup>2</sup> Isopropanol used as the solvent.

<sup>3</sup> Percent P<sub>4</sub>S<sub>3</sub> based on weight of unsaturated hydrocarbon.

As is indicated by the above analyses, the refluxed products from sulfochlorination of an olefin having seven carbon atoms were found to have a sulfur content in the general range of 28 to 31% based on total weight and a higher phosphorus content than was obtained with a sodium hydroxide neutralized product which has been prepared using an equal amount of phosphorus sulfide and which has not been refluxed. The phosphorus and sulfur content of the isopropanol-water refluxed products is considerably higher than that of NaOH neutralized products prepared from the same relative amounts of phosphorus and sulfur without isopropanol-water refluxing.

Another characteristic of the products formed by our process is high chlorine content. This property is most important from the standpoint of use of the products in cutting oils. Although labile chlorine is substantially removed from the products by the reflux step, combined chlorine in the products is present in unusually large quantities for compositions which also have such a high sulfur content. The light color of the products from our process, unusual in high chlorine and sulfur containing compositions, is another advantage in their use particularly in cutting oils.

A single reflux for from about one-half to three hours is usually sufficient to eliminate the bulk of unreacted inorganic ingredients. However, two washings in the reflux are more adequate and are preferred and three or more washings may be used.

After refluxing has been completed, the aqueous layer from the reflux step is separated from the refluxed product. The refluxed product may be blown with air or an inert gas or may be air evaporated to remove low molecular weight unreacted hydrocarbons and other impurities and no filtering of the product is necessary. Small amounts of water in the product may be removed with a drying agent. When blowing with an inert gas we prefer to use nitrogen although any such inert gas may be conveniently employed. The length of time required for removal of the olefins by blowing with air or an inert gas will depend upon the amount of air or inert gas used, the amount of product to be blown and the amount of unreacted olefins and other impurities present in the product. Air evaporation may take as long as 144 hours to remove impurities from the product. However, this period can be substantially lessened by partially finishing the product by blowing with inert gas before air evaporation. When high molecular weight hydrocarbons, such as polymers, are used, blowing and evaporation is not absolutely necessary because traces of water may be eliminated with a drying agent.

As illustrations only and not intended to be limitations upon the scope of this invention, the following are offered as examples of the practice of this invention.

## Example A

1500 g. of C<sub>7</sub> olefin prepared by the polymerization of propylene with butylenes were reacted with 1050 g. (.52 mole per mole of C<sub>7</sub> olefin) of S<sub>2</sub>Cl<sub>2</sub> in the presence of 150 g. of water and 150 g. (.045 mole per mole of C<sub>7</sub> olefin) of P<sub>2</sub>S<sub>5</sub> in a nitrogen atmosphere. The reaction was started at a temperature of 4° C. and was allowed to proceed at a temperature no higher than 42° C. for four hours and thirty-five minutes. The resulting sulfo-chlorinated product was refluxed in the presence of 750 ccs. of a mixture of 50% water and 50% isopropanol at a temperature ranging from 80° C. to 90° C. for a period of two hours. The aqueous phase was removed from the reactants and 375 ccs. of a mixture of 80% water and 20% isopropanol were immediately added. The reactants were subjected to a second reflux at approximately the same temperatures as the first reflux for a period of one hour. The aqueous phase was removed from the product and the product was blown with N<sub>2</sub> for 8 hours and left exposed to air for 89 hours to allow the unreacted olefin to evaporate. The final yield of product was 1912 gm. or 127%.

## Example B

1,000 g. of a C<sub>7</sub> olefin prepared by the polymerization of propylene with butylenes were reacted with 700 g. (.52 mole per mole of C<sub>7</sub> olefin) of S<sub>2</sub>Cl<sub>2</sub> in the presence of 100 g. of water and 100 g. (.045 mole per mole of C<sub>7</sub> olefin) of P<sub>2</sub>S<sub>5</sub>. The reaction was started at a temperature of 10° C. and was allowed to proceed at a temperature no higher than 24° C. for 2 hours and twenty-five minutes. The resulting sulfochlorinated product was refluxed in the presence of 500 ccs. of a mixture of 50% water and 50% isopropanol at a temperature ranging from 80° C. to 90° C. for a period of two hours. The aqueous phase was removed from the reactants and 250 ccs. of a mixture of 80% water and 20% isopropanol were immediately added. The reactants were subjected to a second reflux at approximately the same temperatures for a period of one hour. The aqueous phase was removed from the product and the product was blown with air to remove unreacted olefin. A final yield of 1333 g. or 133% was obtained.

## Example C

1000 g. of C<sub>7</sub> olefin prepared by the polymerization of propylene with butylenes were reacted with 700 g. (.52 mole per mole of C<sub>7</sub> olefin) of S<sub>2</sub>Cl<sub>2</sub> in the presence of 100 g. of water and 50 g. (.023 mole per mole of C<sub>7</sub> olefin) of P<sub>4</sub>S<sub>3</sub> in a nitrogen atmosphere. The reaction was started at a temperature of 10° C. and was allowed to proceed at a temperature no higher than 33° C. for two hours and fifteen minutes. The resulting sulfo-chlorinated product was refluxed in the presence of 500 ccs. of a mixture of 50% water and 50% isopropanol at a temperature ranging from 80° C. to 90° C. for a period of two hours. The aqueous phase was removed from the reactants and 250 ccs. of a mixture of 80% water and 20% isopropanol were immediately added. The reactants were subjected to a second reflux at approximately the same temperatures as the first reflux for a period of one hour. The aqueous phase was removed from the product and the product was blown with nitrogen for 24 hours and left exposed to air for 16 hours to allow the unreacted olefin to evaporate. The final yield of product was 1229 g. or 123%.

## Example D

1000 g. of a C<sub>7</sub> olefin prepared by the polymerization of propylene with butylenes were reacted with 700 g. (.52 mole per mole of C<sub>7</sub> olefin) of S<sub>2</sub>Cl<sub>2</sub> in the presence of 100 g. of water and 50 g. (.023 mole per mole of

$C_7$  olefin) of  $P_4S_3$  in a nitrogen atmosphere. The reaction was started at a temperature of  $10^\circ C$ . and was allowed to proceed at a temperature no higher than  $32^\circ C$ . for 2 hours and fifteen minutes. The resulting sulfochlorinated product was refluxed in the presence of 500 ccs. of a mixture of 50% water and 50% isopropanol at a temperature ranging from  $80^\circ C$ . to  $90^\circ C$ . for a period of two hours. The aqueous phase was removed from the reactants and 250 ccs. of a mixture of 80% water and 20% isopropanol were immediately added. The reactants were subjected to a second reflux at approximately the same temperatures for a period of one hour. The aqueous phase was removed from the product and the product was blown with nitrogen for 24 hours and left exposed to air for 16 hours to allow the unreacted olefins to evaporate. The final yield of 1196 g. or 120% was obtained.

*Example E*

1000 g. of  $C_7$  olefin prepared by the polymerization of propylene with butylenes were reacted with 700 g. (.52 mole per mole of  $C_7$  olefin) of  $S_2Cl_2$  in the presence of 100 g. of water and 50 g. (.023 mole per mole of  $C_7$  olefin) of  $P_4S_3$  in a nitrogen atmosphere. The reaction was started at a temperature of  $15^\circ C$ . and was allowed to proceed at a temperature no higher than  $26^\circ C$ . for 2 hours and thirty minutes. The resulting sulfochlorinated product was refluxed in the presence of 500 ccs. of a mixture of 50% water and 50% acetone at a temperature ranging from  $60^\circ C$ . to  $70^\circ C$ . for a period of two hours. The aqueous phase was removed from the reactants and 250 ccs. of a mixture of 80% water and 20% acetone were immediately added. The reactants were subjected to a second reflux at approximately the same temperatures as the first reflux for a period of one hour. The aqueous phase was removed from the product and the product was blown with nitrogen for 14 hours to remove unreacted olefin. The final yield of product was 1148 g. or 115%.

*Example F*

1000 g. of a  $C_7$  olefin prepared by the polymerization of propylene with butylenes were reacted with 700 g. (.52 mole per mole of  $C_7$  olefin) of  $S_2Cl_2$  in the presence of 100 g. of water and 50 g. (.023 mole per mole of  $C_7$  olefin) of  $P_4S_3$  in a nitrogen atmosphere. The reaction was started at a temperature of  $10^\circ C$ . and was allowed to proceed at a temperature no higher than  $33^\circ C$ . for 2 hours and twenty-seven minutes. The resulting sulfochlorinated product was refluxed in the presence of 500 ccs. of a mixture of 50% water and 50% isopropanol at a temperature ranging from  $80^\circ C$ . to  $90^\circ C$ . for a period of two hours. The aqueous phase was removed from the reactants and 250 ccs. of a mixture of 80% water and 20% isopropanol were immediately added. The reactants were subjected to a second reflux at approximately the same temperatures for a period of one hour. The aqueous phase was removed from the product and the product was exposed to air for 64 hours to allow the unreacted olefin to evaporate. A final yield of 1243 g. or 124% was obtained.

*Example G*

1000 g. of  $C_7$  olefin prepared by the polymerization of propylene with butylenes were reacted with 700 g. (.52 mole per mole of  $C_7$  olefin) of  $S_2Cl_2$  in the presence of 100 g. of water and 50 g. (.023 mole per mole of  $C_7$  olefin) of  $P_4S_3$  in a nitrogen atmosphere. The reaction was started at a temperature of  $4^\circ C$ . and was allowed to proceed at a temperature no higher than  $34^\circ C$ . for two hours and twenty-five minutes. The resulting sulfochlorinated product was refluxed in the presence of 500 ccs. of a mixture of 50% water and 50% isopropanol at a temperature ranging from  $80^\circ C$ . to  $90^\circ C$ . for a period of two hours. The aqueous phase was removed from the reactants and 250 ccs. of a mixture of

80% water and 20% isopropanol were immediately added. The reactants were subjected to a second reflux at approximately the same temperatures as the first reflux for a period of 30 minutes. The aqueous phase was removed and 250 ccs. of the 80% water and 20% isopropanol mixture were added and a third reflux was conducted under about the same conditions for 30 minutes. The aqueous phase was removed from the product and the product was blown with nitrogen for 13 hours to remove unreacted olefin. The final yield of product was 1157 g. or 116%.

*Example H*

1500 g. of a  $C_7$  olefin prepared by the polymerization of propylene with butylenes were reacted with 1050 g. (.52 mole per mole of  $C_7$  olefin) of  $S_2Cl_2$  in the presence of 150 g. of water and 75 g. (.023 mole per mole of  $C_7$  olefin) of  $P_4S_3$  in a nitrogen atmosphere. The reaction was started at a temperature of  $3^\circ C$ . and was allowed to proceed at a temperature no higher than  $64^\circ C$ . for 4 hours and twenty-five minutes. The resulting sulfochlorinated product was refluxed in the presence of 750 ccs. of a mixture of 50% water and 50% isopropanol at a temperature ranging from  $80^\circ C$ . to  $90^\circ C$ . for a period of one hour. The aqueous phase was removed from the reactants and 375 ccs. of a mixture of 80% water and 20% isopropanol were immediately added. The reactants were subjected to a second reflux at a temperature ranging from  $80^\circ C$ . to  $90^\circ C$ . for a period of one hour. The aqueous phase was removed from the product and the product was exposed to air for 144 hours to allow unreacted olefin to evaporate. A final yield of 1627 g. or 108% was obtained.

*Example I*

1500 g. of  $C_{12}$  propylene tetramer prepared by the polymerization of propylene were reacted with 630 g. (.52 mole per mole of  $C_{12}$  tetramer) of  $S_2Cl_2$  in the presence of 150 g. of water and 75 g. (.038 mole per mole of  $C_{12}$  tetramer) of  $P_4S_3$  in a nitrogen atmosphere. The resulting sulfochlorinated product was refluxed in the presence of 750 ccs. of a mixture of 50% water and 50% isopropanol at a temperature ranging from  $80^\circ C$ . to  $90^\circ C$ . for a period of one hour. The aqueous phase was removed from the reactants and 375 ccs. of a mixture of 80% water and 20% isopropanol were immediately added. The reactants were subjected to a second reflux at a temperature ranging from  $80^\circ C$ . to  $90^\circ C$ . for a period of one hour. The aqueous phase was removed from the product and the product was blown with nitrogen to partially remove unreacted olefin. The final product weighed 1851 g. or 123% yield, and contained some unreacted olefins.

*Example J*

1500 g. of a  $C_7$  olefin prepared by the polymerization of propylene with butylenes were reacted with 1050 g. (.52 mole per mole of  $C_7$  olefin) of  $S_2Cl_2$  in the presence of 150 g. of water and 15 g. (.0045 mole per mole of  $C_7$  olefin) of  $P_2S_5$  in a nitrogen atmosphere. The reaction was started at a temperature of  $3^\circ$  and was allowed to proceed at a temperature no higher than  $35^\circ C$ . for 4 hours and thirty-five minutes. The resulting sulfochlorinated product was refluxed in the presence of 750 ccs. of a mixture of 50% water and 50% isopropanol at a temperature ranging from  $80^\circ C$ . to  $90^\circ C$ . for a period of one hour. The aqueous phase was removed from the reactants and 375 cc. of a mixture of 80% water and 20% isopropanol were immediately added. The reactants were subjected to a second reflux at approximately the same temperatures for a period of one hour. The aqueous phase was removed from the product and the product was blown with nitrogen for 10 hours and exposed to air for 16 hours to allow evaporation of unreacted olefin. A final yield of 1836 g. of 122% was obtained.

## Example K

1000 g. of  $C_7$  olefin prepared by the polymerization of propylene with butylenes were reacted with 700 g. (.52 mole per mole of  $C_7$  olefin) of  $S_2Cl_2$  in the presence of 100 g. of water. The reaction was started at a temperature of 10° C. and was allowed to proceed at a temperature no higher than 22° C. for one hour and forty-five minutes. The resulting sulfochlorinated product was refluxed in the presence of 500 ccs. of a mixture of 50% water and 50% isopropanol at a temperature ranging from 80° C. to 90° C. for a period of two hours. The aqueous phase was removed from the reactants and 250 ccs. of a mixture of 80% water and 20% isopropanol were immediately added. The reactants were subjected to a second reflux at approximately the same temperatures as the first reflux for a period of one hour. The aqueous phase was removed from the product and the product was blown with air for 20 hours to remove unreacted olefin. The final yield of product was 1162 g. or 116%.

## Example L

1500 g. of a  $C_{12}$  propylene tetramer prepared by the polymerization of propylene were reacted with 630 g. (.52 mole per mole of  $C_{12}$  tetramer) of  $S_2Cl_2$  in the presence of 150 g. of water and 15 g. (.0076 mole per mole of  $C_{12}$  tetramer) of  $P_2C_5$  in a nitrogen atmosphere. The reaction was started and was allowed to proceed violently as a runaway reaction with reactants spilling from the reaction vessel. The resulting sulfochlorinated product was refluxed in the presence of 750 ccs. of a mixture of 50% water and 50% isopropanol at a temperature ranging from 80° C. to 90° C. for a period of one hour. The aqueous phase was removed from the reactants and 375 ccs. of a mixture of 80% water and 20% isopropanol were immediately added. The reactants were subjected to a second reflux at approximately the same temperatures for a period of one hour. The aqueous phase was removed from the product and the product was blown with nitrogen to remove unreacted olefin. Final yield could not be determined because of spilling over of reactants during the sulfochlorination step.

## Example M

1000 g. of  $C_7$  olefin prepared by the polymerization of propylene with butylenes were reacted with 700 g. (.52 mole per mole of  $C_7$  olefin) of  $S_2Cl_2$ . The reaction was started at a temperature of 10° C. and was allowed to proceed at a temperature no higher than 45° C. for 2 hours and twenty-three minutes. The resulting sulfochlorinated product was refluxed in the presence of 500 ccs. of a mixture of 50% water and 50% isopropanol at a temperature ranging from 80° C. to 90° C. for a period of two hours. The aqueous phase was removed from the reactants and 250 ccs. of a mixture of 80% water and 20% isopropanol were immediately added. The reactants were subjected to a second reflux at approximately the same temperatures as the first reflux for a period of one hour. The aqueous phase was removed from the product and an interim sample of 200 g. was taken out. The remainder of the product was blown with air for 24 hours to remove unreacted olefin. The final yield of the remainder of product was 1031 g.

## Example N

500 g. of a partially linearly unsaturated polymer having a molecular weight of about 750 were reacted with 70 g. (.78 mole per mole of polymer) of  $S_2Cl_2$  in the presence of 25 g. (.17 mole per mole of polymer) of  $P_4S_3$  in a nitrogen atmosphere. The reaction was started at a temperature of 32° C. and was allowed to proceed at a temperature no higher than 73° C. for 2 hours and fifty minutes. The resulting sulfochlorinated product was refluxed in the presence of 250 ccs. of a mixture of 50% water and 50% isopropanol at a temperature ranging from 80° C. to 90° C. for a period of one hour. The

aqueous phase was drained from the product and a 200 g. aliquot was taken and dried on a steam bath. The remainder of the product was dissolved in a solvent, filtered through paper to free it from inorganic-containing solids and after evaporation of the solvent, the remainder of the product was mixed with the dried aliquot. The final total yield was 520 g. or 104%.

## Example O

- 10 500 g. of a partially linearly unsaturated polymer having a molecular weight of about 750 in the presence of 500 ccs. of a naphtha diluent to cut the viscosity of the polymer were reacted with 70 g. (.78 mole per mole of polymer) of  $S_2Cl_2$  in the presence of 25 g. (.17 mole per mole of polymer) of  $P_4S_3$  in a nitrogen atmosphere. The reaction was started at a temperature of 31° C. and was allowed to proceed at a temperature not exceeding 77° C. for a period of 2 hours and fifty minutes. The resulting sulfochlorinated product was refluxed in the presence of 250 ccs. of a mixture of 50% water and 50% isopropanol at a temperature ranging from 61° C. to 77° C. for a period of one hour. The reflux in this example, as in the above examples, was carried out at total reflux temperature and the lower total reflux temperature in this example is attributable to the presence of the naphtha. The aqueous phase was removed from the reactants and 125 ccs. of a mixture of 80% water and 20% alcohol were immediately added. Total reflux was repeated for one hour and the aqueous phase was separated from the product. The product was blown with nitrogen to remove occluded naphtha but unreacted polymer was not removed. The final product was recovered by filtering over a Buchner funnel, removing water by drying with anhydrous  $Na_2SO_4$  in the presence of benzene and evaporating on a steam bath to remove the added volatiles. In the multiple step product recovery, some product was lost; however 468 g. of product were recovered.
- 20 In all of the above examples, a silicone polymer anti-foam agent was used to prevent excessive foaming during sulfochlorination.
- 25 The products from the above examples were analyzed for sulfur content, chlorine content, phosphorus content and NPA color. The results are given in Table II.
- 30
- 35
- 40

45 TABLE II  
PRODUCT ANALYSIS

| Product                | Sulfur, Wt. Percent | Chlorine, Wt. Percent | Phosphorus, Wt. Percent | NPA Color |
|------------------------|---------------------|-----------------------|-------------------------|-----------|
| Example A              | 29.4                | 7.52                  | 1.32                    | 3         |
| Example B              | 25.4                | 9.5                   | 1.03                    | 1½-2      |
| Example C              | 28.2                | 8.54                  | 1.00                    | 1½-2      |
| Example D              | 29.0                | 8.56                  | 0.91                    | 1½-2      |
| Example E              | 28.0                | 11.48                 | 0.24                    | 1½-2      |
| Example F              | 27.4                | 9.06                  | 1.00                    | 1½-2      |
| Example G              | 29.2                | 7.66                  | 0.82                    | 2-2½      |
| Example H              | 30.6                | 7.98                  | 0.61                    | 3-3½      |
| Example I              | 15.1                | 3.1                   | 0.77                    | 1 4       |
| Example J              | 24.2                | 11.3                  | 0.12                    | 4-4½      |
| Example K              | 25.8                | 10.6                  | 0.00                    | 4½-5      |
| Example L              | 19.0                | 4.1                   | 0.15                    | 1 6       |
| Example M              | 25.8                | 11.0                  | 0.00                    | 7         |
| Example N <sup>2</sup> | 4.1                 | 0.5                   | 0.40                    | 4-4½      |
| Example O <sup>2</sup> | 2.74                | 0.13                  | 0.54                    | 4-4½      |

<sup>1</sup> In 5% blend or refined paraffin distillate having a viscosity of 80 to 85 SSU at 100° F.

<sup>2</sup> Contains unreacted polymer.

65 Table II demonstrates the high sulfur and high chlorine content and light color of the products of the present invention. The sulfur and chlorine in the compositions formed by the present process are chemically bonded in the product and the sulfur is not physically suspended as in the usual high sulfur content compositions, although it is to be considered within the scope of the present invention to suspend or dissolve additional quantities of sulfur or chlorine additive in the composition prepared by the present process.

70 Further, compositions prepared in accordance with our

invention possess high sulfur activity even when used in gear oil and cutting oil concentrations. Accordingly, the sulfur activity of various additives, prepared by treating a C<sub>7</sub> olefin with sulfur chloride in the presence of water and phosphorus sulfide and refluxing the product in the presence of an isopropanol-water mixture, was determined in blends of 2% by weight of the additive in an SAE 50 grade mineral oil. The procedure used in determining sulfur activity was that described by me in a paper which I presented at the 1958 meeting of the American Society of Lubricating Engineers, in Cleveland, Ohio, and published in Lubrication Engineering, volume 14, No. 10, pp. 435 to 438 (1958). Briefly the procedure used is as follows: weighed clean copper strips were immersed in 15 g. of the 2% blends in test tubes for 16 hours at temperatures of 200° F., 250° F. and 300° F.; the copper strips were removed, washed with hexane and acetone and immersed for 3 minutes in a 10% potassium cyanide solution which selectively dissolves the reaction products on the strip without appreciably attacking the underlying copper strip itself; the strips were then weighed to determine the mg. weight loss as a measure of the sulfur activity. The results are compared in Table III with the results of the same sulfur activity test conducted with the SAE 50 grade mineral blending oil alone and with a 5% blend of sperm oil containing 10 to 13% sulfur.

TABLE III

| Treatment During Sulfochlorination            |                               |                               | Refluxed<br>Alcohol/<br>H <sub>2</sub> O | Percent<br>Phos.<br>in<br>Prod. | Sulfur Activity of 2%<br>Blends in Oil Mg.<br>Copper Loss in 16 hrs.<br>at ° F. |     |     |
|-----------------------------------------------|-------------------------------|-------------------------------|------------------------------------------|---------------------------------|---------------------------------------------------------------------------------|-----|-----|
| Gm. used for 100 gm.<br>C <sub>7</sub> Olefin |                               |                               |                                          |                                 | 200                                                                             | 250 | 300 |
| H <sub>2</sub> O                              | P <sub>2</sub> S <sub>5</sub> | P <sub>4</sub> S <sub>3</sub> |                                          |                                 |                                                                                 |     |     |
| 10                                            | <sup>1</sup> 10               | None                          | Yes-----                                 | 1.20                            | 20                                                                              | 220 | 332 |
| 10                                            | None                          | <sup>2</sup> 5                | Yes-----                                 | 0.80                            | 22                                                                              | 226 | 292 |
| 10                                            | <sup>2</sup> 2                | None                          | Yes-----                                 | 0.26                            | 35                                                                              | 156 | 212 |
| 10                                            | <sup>3</sup> 1                | None                          | Yes-----                                 | 0.12                            | 68                                                                              | 185 | 233 |
| 5% Sperm Oil (Sulfur Content: 10-13%)-----    |                               |                               |                                          |                                 | 1.5                                                                             | 3.5 | 32  |
| Mineral Blending Oil (No added Sulfur)-----   |                               |                               |                                          |                                 | 1.0                                                                             | 2.0 | 2.5 |

<sup>1</sup> 0.045 moles.<sup>2</sup> 0.023 moles.<sup>3</sup> 0.012 moles.

The data in Table III demonstrates the high sulfur activity of the compositions prepared in accordance with our invention under conditions of use at low temperatures, such as for use in gear oils.

The use of the solvent-water reflux step in accordance with the present invention vastly improved the color stability of the product and additional improvement in color stability was found to accompany the presence of a phosphorus compound in the product. Reaction products prepared in accordance with the present invention using a C<sub>7</sub> olefin as the unsaturated hydrocarbons were submitted to a temperature of 130° F. for a period of 26 days and the true color changes of the products are compared with products of other processes as indicated in Table IV below.

The data in Table IV demonstrate the increased product color stability obtainable from the use of our present invention. The C<sub>7</sub> olefin, sulfochlorinated in the presence of phosphorus pentasulfide and alcohol-water refluxed, exhibits excellent color stability when aged for 26 days at 130° F., equivalent to aging for approximately one year at room temperatures. When the product was sodium hydroxide neutralized but not refluxed, the true color was substantially increased after aging, thereby demonstrating inferior color stability. When phosphorus pentasulfide and water was eliminated separately from the compositions, the color stability also decreased somewhat. When both phosphorus pentasulfide and water were eliminated, another substantial decrease in color stability occurred.

Concerning the refluxed compositions, as set out in Table IV, it is important to note that even the refluxed product (No. II) having a very low phosphorus content (0.12%) exhibited excellent color stability on aging.

Compositions prepared from C<sub>7</sub> olefins by the present process and submitted to temperatures of 130° F. for 26 days were then cut back to a 3% blend with a refined paraffin distillate having a viscosity of 80 to 85 SSU at 100° F. to simulate practical cutting oil concentrations.

The 3% blends were found to have unusually light color, generally in the NPA color range of from 2 to 3½.

The sulfochlorinated hydrocarbons produced by the present invention are particularly useful in cutting oils where high sulfur and chlorine activity, light color, and color stability are of great importance. The sulfochlorinated products may also be used as additives for automotive gear oils where it is desirable to incorporate sulfur compositions to pass shock load tests and are applicable to many other situations within the skill of the art.

An important advantage of the present process is the production of high sulfur, chlorine containing hydrocarbons having light color and suitable for commercial use. Another advantage is the reduction in the amount of time necessary for producing a finished sulfochlorinated composition. Other advantages will appear evident to one skilled in the art from the above disclosures and descriptions. While we have described in detail the preferred embodiment of the present invention, it will be apparent to those skilled in the art that certain modifications thereto are possible so that it is understood that the present invention is not intended to be limited to the details set forth above, but includes within its scope such modifications as come within the scope of the appended claims.

We claim:

1. In a process for the sulfochlorination of linearly unsaturated hydrocarbons the steps comprising reacting a linearly unsaturated hydrocarbon with a sulfur chloride and refluxing the resulting sulfochlorinated hydrocarbon in the presence of substantial portions of a mixture of water and an oxygen-containing essentially non-reacting water-miscible organic compound wherein the water and oxygen-containing compound in said mixture are each

TABLE IV

| No.                   | Treatment During Sulfochlorination |                                            |                                               | NaOH<br>Neutralized | Product After Preparation |              |               | After Exposure at<br>130° F. for— |                           |
|-----------------------|------------------------------------|--------------------------------------------|-----------------------------------------------|---------------------|---------------------------|--------------|---------------|-----------------------------------|---------------------------|
|                       | H <sub>2</sub> O <sup>1</sup>      | P <sub>2</sub> S <sub>5</sub> <sup>2</sup> | Refluxed<br>Isopro-<br>panol/H <sub>2</sub> O |                     | Per-<br>cent P            | NPA<br>Color | True<br>Color | 13 days—<br>True<br>Color         | 26 days—<br>True<br>Color |
| I-----                | 10                                 | .045                                       | Yes-----                                      | No-----             | 1.20                      | 3            | 12            | 100                               | 132                       |
| II <sup>3</sup> ----- | 10                                 | .0045                                      | Yes-----                                      | No-----             | 0.12                      | 4-4½         | 33            | 264                               | 380                       |
| III-----              | 10                                 | .045                                       | No-----                                       | Yes-----            | 0.05                      | 4½           | 46            | 460                               | 992                       |
| IV-----               | None                               | .045                                       | No-----                                       | Yes-----            | 0.05                      | 4½-5         | 60            | 528                               | 1,214                     |
| V-----                | 10                                 | None                                       | No-----                                       | Yes-----            | None                      | 4-4½         | 33            | 528                               | 1,156                     |
| VI-----               | None                               | None                                       | No-----                                       | Yes-----            | None                      | 4-4½         | 33            | 1,150                             | 1,856                     |

<sup>1</sup> Grams per 100 grams C<sub>7</sub> olefin.<sup>2</sup> Moles per mole of C<sub>7</sub> olefin.<sup>3</sup> Represents a composite of many batches of C<sub>7</sub> olefin sulfochlorinated in the presence of water.

present in substantial percents at the total refluxing temperature, said oxygen-containing compound boiling below about 100° C.

2. The process of claim 1 wherein the oxygen-containing essentially non-reacting water-miscible organic compound boils within the range of 50 to 100° C.

3. The process of claim 1 wherein the oxygen-containing essentially non-reacting water-miscible organic compound is a water-miscible alcohol.

4. The process of claim 1 wherein the oxygen-containing essentially non-reacting water-miscible organic compound is isopropanol.

5. The process of claim 1 wherein the oxygen-containing essentially non-reacting water-miscible organic compound is a water-miscible ketone.

6. The process of claim 1 wherein the oxygen-containing essentially non-reacting water-miscible organic compound is acetone.

7. The process of claim 1 wherein the total refluxing temperature is in the range of from about 50° C. to about 100° C.

8. The process of claim 1 wherein the linearly unsaturated hydrocarbon is a polymer.

9. The process of claim 1 wherein the linearly unsaturated hydrocarbon is reacted with from 0.3 to 2.0 moles of sulfur chloride per mole of linearly unsaturated hydrocarbon.

10. The process of claim 1 wherein the sulfur chloride is sulfur mono-chloride.

11. The process of claim 1 wherein the sulfur chloride treatment is carried out in the presence of water.

12. The process of claim 1 wherein the sulfur chloride treatment is carried out in the presence of a phosphorus sulfide.

13. A method for producing high sulfur-containing compositions of light color and high color stability which comprises the steps of reacting a linearly unsaturated hydrocarbon with sulfur chloride in the presence of 1 to 50 volume percent water, and refluxing the resulting reaction product in the presence of substantial portions of a mixture of water-miscible alcohol and water wherein the water and oxygen-containing compound in said mixture are each present in substantial percents at the total refluxing temperature for at least 10 minutes.

14. A method for producing high sulfur and phosphorus-containing compositions of light color and high color stability which comprises the steps of adding to a linearly unsaturated hydrocarbon from about .0025 to about 0.2 mole of phosphorus sulfide per mole of linearly unsaturated hydrocarbon, treating said linearly unsaturated hydrocarbon and phosphorus sulfide with sulfur chloride, and refluxing the reaction mixture in the presence of substantial portions of a mixture of water-miscible alcohol and water wherein the water and alcohol in said mixture are each present in substantial percents at the total refluxing temperature for at least 10 minutes.

15. The process of claim 14 in which the phosphorus sulfide is  $P_2S_5$ .

16. A method for producing high sulfur and phosphorus containing compositions of light color and high color stability which comprises the steps of adding to a linearly unsaturated hydrocarbon from about .0025 to about 0.2 mole of phosphorus sulfide per mole of linearly unsaturated hydrocarbon, incrementally treating said linearly unsaturated hydrocarbon and phosphorus sulfide with 0.3 to 2.0 moles of sulfur chloride per mole of linearly unsaturated hydrocarbon in the presence of 1 to 50 volume percent water so as not to exceed the boiling point of the reaction mixture, and refluxing the reaction mixture in the presence of substantial portions of a water-miscible alcohol and water wherein the water and alcohol in said mixture are each present in substantial percents at the total refluxing temperature for at least 10 minutes.

17. A process for sulfochlorinating linearly unsaturated hydrocarbons which comprises the steps of incrementally treating a linearly unsaturated hydrocarbon with from about 0.3 to about 2.0 moles of sulfur chloride per mole of linearly unsaturated hydrocarbon, maintaining the reaction at a temperature not exceeding about 90° C., adding substantial portions of a first mixture of a water-miscible alcohol and water to the reactants, refluxing the mixture at the total refluxing temperature, separating a water layer from the reactants, adding substantial portions of a second mixture of a water-miscible alcohol and water to the reactants, repeating the refluxing at the total refluxing temperature, separating a water layer from the reactants, and removing unreacted linearly unsaturated hydrocarbons from the reactants, wherein the water and alcohol in said first and second mixtures are each present in substantial percents.

18. The product formed by the process of claim 1.

19. The product formed by the process of claim 14.

20. The product formed by the process of claim 16.

21. A method for producing high sulfur-containing compositions of light color and high color stability, which method comprises the steps of reacting a linearly unsaturated hydrocarbon with a sulfur chloride and refluxing the resulting sulfochlorinated hydrocarbon in the presence of about 500 milliliters of a mixture of water and an oxygen-containing essentially non-reacting water-miscible organic compound boiling in the range of 50 to 100° C. per 1000 grams of said linearly unsaturated hydrocarbon, said refluxing being at the reflux temperature of said mixture.

50  
22. The product formed by the process of claim 21.

23. The product formed by the process of claim 22.

24. The product formed by the process of claim 23.

25. The product formed by the process of claim 24.

26. The product formed by the process of claim 25.

27. The product formed by the process of claim 26.

28. The product formed by the process of claim 27.

29. The product formed by the process of claim 28.

30. The product formed by the process of claim 29.

31. The product formed by the process of claim 30.

32. The product formed by the process of claim 31.

33. The product formed by the process of claim 32.

34. The product formed by the process of claim 33.

35. The product formed by the process of claim 34.

36. The product formed by the process of claim 35.

37. The product formed by the process of claim 36.

38. The product formed by the process of claim 37.

39. The product formed by the process of claim 38.

40. The product formed by the process of claim 39.

41. The product formed by the process of claim 40.

42. The product formed by the process of claim 41.

43. The product formed by the process of claim 42.

44. The product formed by the process of claim 43.

45. The product formed by the process of claim 44.

46. The product formed by the process of claim 45.

47. The product formed by the process of claim 46.

48. The product formed by the process of claim 47.

49. The product formed by the process of claim 48.

50. The product formed by the process of claim 49.

51. The product formed by the process of claim 50.

52. The product formed by the process of claim 51.

53. The product formed by the process of claim 52.

54. The product formed by the process of claim 53.

55. The product formed by the process of claim 54.

References Cited in the file of this patent

UNITED STATES PATENTS

2,708,199 Eby ----- May 10, 1955  
2,727,030 Beretvas ----- Dec. 13, 1955  
2,853,480 Lindert ----- Sept. 23, 1958